# EUROPEAN PATENT APPLICATION

(11) **EP 2 267 545 A1**
(43) Date of publication of application: **29.12.2010**
(21) Application number: 10167041.2
(22) Date of filing: 23.06.2010
(51) Int. Cl.: G03G 9/08, G03G 9/087, G03G 9/093

(54) **Toner compositions**

(30) Priority: 24.06.2009 US 491196
(71) Applicant: Xerox Corporation, Rochester, New York 14644 (US)
(72) Inventor: Zhou, Ke, Oakville Ontario L6H 0C6 (CA); Zwartz, Edward G., Mississauga Ontario L5J 4B2 (CA); McDougall, Maria N V., Oakville Ontario L6L 6X1 (CA); Pawlak, John, Rochester, NY 14625 (US); Gerroir, Paul J., Oakville Ontario L6L 1P9 (CA); Moffat, Karen A., Brantford Ontario N3R 7P8 (CA); Veregin, Richard P N., Mississauga Ontario L5L 5T6 (CA)
(74) Representative: De Anna, Pier Luigi

(57) **Abstract**

A toner including at least one amorphous polyester, at least one crystalline polyester and at least one ester wax, wherein the at least one amorphous polyester and the at least one ester wax have a difference in solubility parameter of from about 0.1 to about 1.7.

## Description

### BACKGROUND

The present invention relates to toners suitable for electrophotographic apparatuses.

Numerous processes are within the purview of those skilled in the art for the preparation of toners. Emulsion aggregation (EA) is one such method. EA toners may be formed by aggregating a colorant with a latex polymer formed by emulsion polymerization. For example, U.S. Patent No. 5,853,943, is directed to a semi-continuous emulsion polymerization process for preparing a latex by first forming a seed polymer. Other examples of emulsion/aggregation/coalescing processes for the preparation of toners are illustrated in U.S. Patent Nos. 5,403,693, 5,418,108, 5,364,729, and 5,346,797. Other processes are disclosed in U.S. Patent Nos. 5,527,658, 5,585,215, 5,650,255, 5,650,256 and 5,501,935.

The appropriate components and process aspects of the each of the foregoing U. S. Patents and Patent Publications may be selected for the present disclosure in embodiments thereof.

Polyester EA ultra low melt (ULM) toners have been prepared utilizing amorphous and crystalline polyester resins. While these toners may exhibit excellent fusing properties including crease minimum fixing temperature (MFT) and fusing latitude, peak gloss of these toners may be unacceptably high. These toners may exhibit poor charging characteristics, which may be due to the crystalline resin component migrating to the surface during coalescence, as well as poor toner flow and poor blocking. Improved toners thus remain desirable.

Certain fusing systems use oil as a toner release agent. However, after fusing, oil may leave streaks on the page which may result in image quality issues such as differential gloss and render the prints unusable for certain end-use applications. Waxes have been added to toners for the purpose of aiding in toner release from the fuser roll, for example in low oil or oil-less fuser machines. Use of wax may reduce or eliminate the need for oil. However, successful incorporation of wax has been a challenge for certain toner formulations. There remains a need for improved toners for low oil or oil-less fuser machines. There further remains a need for improved emulsion aggregation toners for low oil or oil-less fuser.

### SUMMARY

The present disclosure provides toners and methods for their production. In embodiments, a toner of the present disclosure may include at least one amorphous polyester, at least one crystalline polyester and at least one ester wax, wherein the amorphous polyester and the at least one ester wax have a difference in solubility parameter of from about 0.1 to about 1.7.

In other embodiments, a toner of the present disclosure may include at least one amorphous polyester, at least one crystalline polyester, at least one ester wax, and one or more optional ingredients selected from the group consisting of colorants, optional additional additives, and combinations thereof; wherein the amorphous polyester and the at least one ester wax have a difference in solubility parameter of from about 0.1 to about 1.7.

Processes of the present disclosure may include, for example, contacting at least one amorphous polyester with at least one crystalline polyester and at least one ester wax in an emulsion comprising at least one surfactant; wherein the amorphous polyester and the at least one ester wax have a difference in solubility parameter of from about 0.1 to about 1.7, and an optional colorant; aggregating the small particles to form a plurality of core particles; contacting the core particles with an additional quantity of at least one amorphous polyester resin to form a shell on the core particles, coalescing the core-shell particles, and optionally recovering the particles.

### DETAILED DESCRIPTION

The present invention provides toner particles having desirable charging, flow, blocking, and gloss properties. In embodiments, the present disclosure provides emulsion aggregation toner particles for low oil or oil-less fuser systems. In embodiments, the toners include incorporation of a wax that is compatible with the matrix toner components. The toner particles may possess a core-shell configuration, with a branched resin or partially cross-linked resin in the core, shell, or both.

Resins

Suitable resins include amorphous low molecular weight linear polyesters, high molecular weight branched and crosslinked polyesters and crystalline polyesters. In embodiments, the polymer utilized to form the resin core may be a polyester resin, including the resins described in U.S. Patent Nos. 6,593,049 and 6,756,176. Suitable resins may also include a mixture of an amorphous polyester resin and a crystalline polyester resin as described in U.S. Patent No. 6,830,860.

In embodiments, the resin may be a polyester resin formed by reacting a diol with a diacid in the presence of an optional catalyst. For forming a crystalline polyester, suitable organic diols include aliphatic diols with from about 2 to about 36 carbon atoms, such as 1,2-ethanediol, 1,3-propanediol, 1,4-butanediol, 1,5-pentanediol, 1,6-hexanediol, 1,7-heptanediol, 1,8-octanediol, 1,9-nonanediol, 1,10-decanediol, 1,12-dodecanediol and the like; alkali sulfo-aliphatic diols such as sodio 2-sulfo-1,2-ethanediol, lithio 2-sulfo-1,2-ethanediol, potassio 2-sulfo-1,2-ethanediol, sodio 2-sulfo-1,3-propanediol, lithio 2-sulfo-1,3-propanediol, potassio 2-sulfo-1,3-propanediol, mixture thereof, and the like. The aliphatic diol may be, for example, selected in an amount of from about 40 to about 60 mole percent, in embodiments from about 42 to about 55 mole percent, in embodiments from about 45 to about 53 mole percent, and the alkali sulfo-aliphatic diol can be selected in an amount of from about 0 to about 10 mole percent, in embodiments from about 1 to about 4 mole percent of the resin.

Examples of organic diacids or diesters including vinyl diacids or vinyl diesters selected for the preparation of the crystalline resins include oxalic acid, malonic acid, succinic acid, glutaric acid, adipic acid, pimelic acid, suberic acid, azelaic acid, sebacic acid, undecanedioic acid, dodecanedioic acid, 1,11-undecane dicarboxylic acid, 1,12-dodecane dicarboxylic acid, 1,13-tridecane dicarboxylic acid, 1,14-tetradecane dicarboxlic acid, fumaric acid, dimethyl fumarate, dimethyl itaconate, cis-1,4-diacetoxy-2-butene, diethyl fumarate, diethyl maleate, phthalic acid, isophthalic acid, terephthalic acid, naphthalene-2,6-dicarboxylic acid, naphthalene-2,7-dicarboxylic acid, cyclohexane dicarboxylic acid, malonic acid and mesaconic acid, a diester or anhydride thereof; and an alkali sulfo-organic diacid such as the sodio, lithio or potassio salt of dimethyl-5-sulfo-isophthalate, dialkyl-5-sulfo-isophthalate-4-sulfo-1,8-naphthalic anhydride, 4-sulfo-phthalic acid, dimethyl-4-sulfo-phthalate, dialkyl-4-sulfo-phthalate, 4-sulfophenyl-3,5-dicarbomethoxybenzene, 6-sulfo-2-naphthyl-3,5-dicarbomethoxybenzene, sulfo-terephthalic acid, dimethyl-sulfo-terephthalate, 5-sulfo-isophthalic acid, dialkyl-sulfo-terephthalate, sulfoethanediol, 2-sulfopropanediol, 2-sulfobutanediol, 3-sulfopentanediol, 2-sulfohexanediol, 3-sulfo-2-methylpentanediol, 2-sulfo-3,3-dimethylpentanediol, sulfo-p-hydroxybenzoic acid, N,N-bis(2-hydroxyethyl)-2-amino ethane sulfonate, or mixtures thereof. The organic diacid may be selected in an amount of, for example, in embodiments from about 40 to about 60 mole percent, in embodiments from about 42 to about 52 mole percent, in embodiments from about 45 to about 50 mole percent, and the alkali sulfo-aliphatic diacid can be selected in an amount of from about 1 to about 10 mole percent of the resin.

Examples of crystalline resins include polyesters, polyamides, polyimides, polyolefins, polyethylene, polybutylene, polyisobutyrate, ethylene-propylene copolymers, ethylene-vinyl acetate copolymers, polypropylene, mixtures thereof, and the like. Specific crystalline resins may be polyester based, such as poly(ethylene-adipate), poly(propylene-adipate), poly(butylene-adipate), poly(pentylene-adipate), poly(hexylene-adipate), poly(octylene-adipate), poly(nonylene-adipate), poly(decylene-adipate), poly(undecylene-adipate), poly(dodecylene-adipate), poly(ethylene-succinate), poly(propylene-succinate), poly(butylene-succinate), poly(pentylene-succinate), poly(hexylene-succinate), poly(octylene-succinate), poly(nonylene-succinate), poly(decylene-succinate), poly(undecylene-succinate), poly(dodecylene-succinate), poly(ethylene-sebacate), poly(propylene-sebacate), poly(butylene-sebacate), poly(pentylene-sebacate), poly(hexylene-sebacate), poly(octylene-sebacate), poly(nonylene-sebacate), poly(decylene-sebacate), poly(undecylene-sebacate), poly(dodecylene-sebacate), poly(ethylene-dodecanedioate), poly(propylene-dodecanedioate), poly(butylene-dodecanedioate), poly(pentylene-dodecanedioate), poly(hexylene-dodecanedioate), poly(octylene-dodecanedioate), poly(nonylene-dodecandioate), poly(decylene-dodecandioate), poly(undecylene-dodecandioate), poly(dodecylene-dodecandioate), poly(ethylene-fumarate), poly(propylene-fumarate), poly(butylene-fumarate), poly(pentylene-fumarate), poly(hexylene-fumarate), poly(octylene-fumarate), poly(nonylene-fumarate), poly(decylene-fumarate), copolymers such as copoly(ethylene-fumarate)-copoly(ethylene-dodecandioate) and the like, alkali copoly(5-sulfoisophthaloyl)-copoly(ethylene-adipate), alkali copoly(5-sulfoisophthaloyl)-copoly(propylene-adipate), alkali copoly(5-sulfoisophthaloyl)-copoly(butylene-adipate), alkali copoly(5-sulfo-isophthaloyl)-copoly(pentylene-adipate), alkali copoly(5-sulfoisophthaloyl)-copoly(hexylene-adipate), alkali copoly(5-sulfo-isophthaloyl)-copoly(octylene-adipate), alkali copoly(5-sulfo-isophthaloyl)-copoly(ethylene-adipate), alkali copoly(5-sulfo-isophthaloyl)-copoly (propylene-adipate), alkali copoly(5-sulfo-isophthaloyl)-copoly(butylene-adipate), alkali copoly(5-sulfoisophthaloyl)-copoly(pentylene-adipate), alkali copoly(5-sulfo-isophthaloyl)-copoly(hexylene-adipate), alkali copoly(5-sulfo-isophthaloyl)-copoly(octylene-adipate), alkali copoly(5-sulfoisophthaloyl)-copoly(ethylene-succinate), alkali copoly(5-sulfoisophthaloyl)-copoly(propylene-succinate), alkali copoly(5-sulfoisophthaloyl)-copoly(butylenes-succinate), alkali copoly(5 -sulfoisophthaloyl)-copoly(pentylene-succinate), alkali copoly(5 -sulfoisophthaloyl)-copoly(hexylene-succinate), alkali copoly(5-sulfoisophthaloyl)-copoly(octylene-succinate), alkali copoly(5-sulfo-isophthaloyl)-copoly(ethylene-sebacate), alkali copoly(5-sulfo-isophthaloyl)-copoly(propylene-sebacate), alkali copoly(5-sulfo-isophthaloyl)-copoly(butylene-sebacate), alkali copoly(5-sulfo-isophthaloyl)-copoly(pentylene-sebacate), alkali copoly(5-sulfo-isophthaloyl)-copoly(hexylene-sebacate), alkali copoly(5-sulfo-isophthaloyl)-copoly(octylene-sebacate), alkali copoly(5-sulfo-isophthaloyl)-copoly(ethylene-adipate), alkali copoly(5-sulfo-isophthaloyl)-copoly(propylene-adipate), alkali copoly(5-sulfo-isophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipate), wherein alkali is a metal like sodium, lithium or potassium. Examples of polyamides include poly(ethylene-adipamide), poly(propylene-adipamide), poly(butylenes-adipamide), poly(pentylene-adipamide), poly(hexylene-adipamide), poly(octylene-adipamide), poly(ethylene-succinamide), and poly(propylene-sebecamide). Examples of polyimides include poly(ethylene-adipimide), poly(propylene-adipimide), poly(butylene-adipimide), poly(pentylene-adipimide), poly(hexylene-adipimide), poly(octylene-adipimide), poly(ethylene-succinimide), poly(propylene-succinimide), and poly(butylene-succinimide).

The crystalline resin may be present, for example, in an amount of from about 5 to about 50 percent by weight of the toner components, in embodiments from about 5 to about 35 percent by weight of the toner components. The crystalline resin can possess various melting points of, for example, from about 30° C to about 120° C, in embodiments from about 50° C to about 90° C. The crystalline resin may have a number average molecular weight (Mn), as measured by gel permeation chromatography (GPC) of, for example, from about 1,000 to about 50,000, in embodiments from about 2,000 to about 25,000, and a weight average molecular weight (Mw) of, for example, from about 2,000 to about 100,000, in embodiments from about 3,000 to about 80,000, as determined by Gel Permeation Chromatography using polystyrene standards. The molecular weight distribution (Mw/Mn) of the crystalline resin may be, for example, from about 2 to about 6, in embodiments from about 2 to about 4.

Examples of diacid or diesters including vinyl diacids or vinyl diesters selected for the preparation of amorphous polyesters include dicarboxylic acids or diesters such as terephthalic acid, phthalic acid, isophthalic acid, fumaric acid, dimethyl fumarate, dimethyl itaconate, cis-1,4-diacetoxy-2-butene, diethyl fumarate, diethyl maleate, maleic acid, succinic acid, itaconic acid, succinic anhydride, dodecylsuccinic acid, dodecylsuccinic anhydride, dodecenylsuccinic acid, dodecenylsuccinic anhydride, glutaric acid, glutaric anhydride, adipic acid, pimelic acid, suberic acid, azelaic acid, dodecane diacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dimethyl dodecylsuccinate, and combinations thereof. The organic diacid or diester may be present, for example, in an amount from about 40 to about 60 mole percent of the resin, in embodiments from about 42 to about 52 mole percent of the resin, in embodiments from about 45 to about 50 mole percent of the resin.

Examples of diols utilized in generating the amorphous polyester include 1,2-propanediol, 1,3-propanediol, 1,2-butanediol, 1,3-butanediol, 1,4-butanediol, pentanediol, hexanediol, 2,2-dimethylpropanediol, 2,2,3-trimethylhexanediol, heptanediol, dodecanediol, bis(hydroxyethyl)-bisphenol A, bis(2-hydroxypropyl)-bisphenol A, 1,4-cyclohexanedimethanol, 1,3-cyclohexanedimethanol, xylenedimethanol, cyclohexanediol, diethylene glycol, bis(2-hydroxyethyl) oxide, dipropylene glycol, dibutylene, and combinations thereof. The amount of organic diol selected can vary, and may be present, for example, in an amount from about 40 to about 60 mole percent of the resin, in embodiments from about 42 to about 55 mole percent of the resin, in embodiments from about 45 to about 53 mole percent of the resin.

In embodiments, the resin may be formed by condensation polymerization methods. Polycondensation catalysts which may be utilized for either the crystalline or amorphous polyesters include tetraalkyl titanates, dialkyltin oxides such as dibutyltin oxide, tetraalkyltins such as dibutyltin dilaurate, and dialkyltin oxide hydroxides such as butyltin oxide hydroxide, aluminum alkoxides, alkyl zinc, dialkyl zinc, zinc oxide, stannous oxide, or combinations thereof. Such catalysts may be utilized in amounts of, for example, from about 0.01 mole percent to about 5 mole percent based on the starting diacid or diester used to generate the polyester resin.

In embodiments, the polyester resin may be a saturated or unsaturated amorphous polyester resin. Illustrative examples of saturated and unsaturated amorphous polyester resins selected for the process and particles of the present disclosure include any of the various amorphous polyesters, such as polyethylene-terephthalate, polypropylene-terephthalate, polybutylene-terephthalate, polypentylene-terephthalate, polyhexalene-terephthalate, polyheptadene-terephthalate, polyoctalene-terephthalate, polyethylene-isophthalate, polypropylene-isophthalate, polybutylene-isophthalate, polypentylene-isophthalate, polyhexalene-isophthalate, polyheptadene-isophthalate, polyoctalene-isophthalate, polyethylene-sebacate, polypropylene sebacate, polybutylene-sebacate, polyethylene-adipate, polypropylene-adipate, polybutylene-adipate, polypentylene-adipate, polyhexalene-adipate, polyheptadene-adipate, polyoctalene-adipate, polyethylene-glutarate, polypropylene-glutarate, polybutylene-glutarate, polypentylene-glutarate, polyhexalene-glutarate, polyheptadene-glutarate, polyoctalene-glutarate polyethylene-pimelate, polypropylene-pimelate, polybutylene-pimelate, polypentylene-pimelate, polyhexalene-pimelate, polyheptadene-pimelate, poly(ethoxylated bisphenol A-fumarate), poly(ethoxylated bisphenol A-succinate), poly(ethoxylated bisphenol A-adipate), poly(ethoxylated bisphenol A-glutarate), poly(ethoxylated bisphenol A-terephthalate), poly(ethoxylated bisphenol A-isophthalate), poly(ethoxylated bisphenol A-dodecenylsuccinate), poly(propoxylated bisphenol A-fumarate), poly(propoxylated bisphenol A-succinate), poly(propoxylated bisphenol A-adipate), poly(propoxylated bisphenol A-glutarate), poly(propoxylated bisphenol A-terephthalate), poly(propoxylated bisphenol A-isophthalate), poly(propoxylated bisphenol A-dodecenylsuccinate), SPAR (Dixie Chemicals), BECKOSOL (Reichhold Inc), ARAKOTE (Ciba-Geigy Corporation), HETRON (Ashland Chemical), PARAPLEX (Rohm & Haas), POLYLITE (Reichhold Inc), PLASTHALL (Rohm & Haas), CYGAL (American Cyanamide), ARMCO (Armco Composites), ARPOL (Ashland Chemical), CELANEX (Celanese Eng), RYNITE (DuPont), STYPOL (Freeman Chemical Corporation) and combinations thereof. The resins can also be functionalized, such as carboxylated, sulfonated, or the like, and particularly such as sodio sulfonated, if desired.

In embodiments, an unsaturated polyester resin may be utilized as a latex resin. Examples of such resins include those disclosed in U.S. Patent No. 6,063,827. Exemplary unsaturated amorphous polyester resins include, but are not limited to, poly(propoxylated bisphenol A co-fumarate), poly(ethoxylated bisphenol A co-fumarate), poly(butyloxylated bisphenol A co-fumarate), poly(copropoxylated bisphenol A co-ethoxylated bisphenol A co-fumarate), poly(1,2-propylene fumarate), poly(propoxylated bisphenol A co-maleate), poly(ethoxylated bisphenol A co-maleate), poly(butyloxylated bisphenol A co-maleate), poly(co-propoxylated bisphenol A co-ethoxylated bisphenol A co-maleate), poly(1,2-propylene maleate), poly(propoxylated bisphenol A co-itaconate), poly(ethoxylated bisphenol A co-itaconate), poly(butyloxylated bisphenol A co-itaconate), poly(copropoxylated bisphenol A co-ethoxylated bisphenol A co-itaconate), poly(1,2-propylene itaconate), and combinations thereof.

In embodiments, a suitable linear amorphous polyester resin may be a poly(propoxylated bisphenol A co-fumarate) resin having the following formula (I):

wherein m may be from about 5 to about 1000.

An example of a linear amorphous propoxylated bisphenol A fumarate resin which may be utilized as a latex resin is available under the trade name SPARII™ from Resana S/A Industrias Quimicas, Sao Paulo Brazil. Other suitable linear amorphous resins include those disclosed in U.S. Patent Nos. 4,533,614, 4,957,774 and 4,533,614, which can be linear polyester resins including dodecylsuccinic anhydride, terephthalic acid, and alkyloxylated bisphenol A. Other alkoxylated bisphenol A terephthalate resins that may be utilized and are commercially available include GTU-FC115, commercially available from Kao Corporation, Japan, and the like.

Suitable crystalline resins include those disclosed in U.S. Patent 7,329,476, U.S. Patent. Application Publication Nos. 2006/0216626, 2008/0107990, 2008/0236446, and 2009/0047593. In embodiments, a suitable crystalline resin may include a resin composed of ethylene glycol and a mixture of dodecanedioic acid and fumaric acid co-monomers with the following formula:

wherein b is from 5 to 2000 and d is from 5 to 2000.

For example, in embodiments, a poly(propoxylated bisphenol A co-fumarate) resin of formula I as described above may be combined with a crystalline resin of formula II to form a core.

In embodiments, the amorphous resin or combination of amorphous resins utilized in the core may have a glass transition temperature of from about 30°C to about 80°C, in embodiments from about 35°C to about 70°C. In further embodiments, the combined resins utilized in the core may have a melt viscosity of from about 10 to about 1,000,000 Pa*S at about 130°C, in embodiments from about 50 to about 100,000 Pa*S.

One, two, or more toner resins may be used. In embodiments where two or more toner resins are used, the toner resins may be in any suitable ratio (e.g., weight ratio) such as for instance about 10% (first resin)/90% (second resin) to about 90% (first resin)/10% (second resin).

In one embodiment, the amorphous polyester resin is present in an amount of from about 50 % to about 85 % by weight based upon the total weight of the toner.

In embodiments, linear amorphous polyesters may be combined with a high molecular weight branched or cross-linked amorphous polyesters to provide improved toner properties such as higher hot offset temperatures and control of print gloss properties. This high molecular weight polyester may include, in embodiments, for example, a branched resin or polymer, a cross-linked resin or polymer, or mixtures thereof, or a non-cross-linked resin that has been subjected to cross-linking. In accordance with the present disclosure, from about 1% by weight to about 100% by weight of the higher molecular weight resin may be branched or cross-linked, in embodiments from about 2% by weight to about 50% by weight of the higher molecular weight resin may be branched or cross-linked. As used herein, the term "high molecular weight resin" refers to a resin wherein the weight-average molecular weight (Mw) of the chloroform-soluble fraction of the resin is above about 15,000 and a polydispersity index (PD) above about 4, as measured by gel permeation chromatography versus standard polystyrene reference resins. The PD index is the ratio of the weight-average molecular weight (Mw) and the number-average molecular weight (Mn).

The high molecular weight amorphous polyester resins may prepared by branching or cross-linking linear polyester resins. Branching agents can be utilized, such as trifunctional or multifunctional monomers, which agents usually increase the molecular weight and polydispersity of the polyester. Suitable branching agents can include glycerol, trimethylol ethane, trimethylol propane, pentaerythritol, sorbitol, diglycerol, trimellitic acid, trimellitic anhydride, pyromellitic acid, pyromellitic anhydride, 1,2,4-cyclohexanetricarboxylic acid, 2,5,7-naphthalenetricarboxylic acid, 1,2,4-butanetricarboxylic acid, combinations thereof, and the like. These branching agents can be utilized in effective amounts of from about 0.1 mole percent to about 20 mole percent based on the starting diacid or diester used to make the resin.

Compositions containing modified polyester resins with a polybasic carboxylic acid which may be utilized in forming high molecular weight polyester resins include those disclosed in U.S. Patent No. 3,681,106, as well as branched or cross-linked polyesters derived from polyvalent acids or alcohols as illustrated in U.S. Patent Nos. 4,298,672; 4,863,825; 4,863,824; 4,845,006; 4,814,249; 4,693,952; 4,657,837; 5,143,809; 5,057,596; 4,988,794; 4,981,939; 4,980,448; 4,960,664; 4,933,252; 4,931,370; 4,917,983 and 4,973,539.

In embodiments, cross-linked polyesters resins may be made from linear polyester resins that contain sites of unsaturation that can react under free-radical conditions. Examples of such resins include those disclosed in U.S. Patent Nos. 5,227,460; 5,376,494; 5,480,756; 5,500,324; 5,601,960; 5,629,121; 5,650,484; 5,750,909; 6,326,119; 6,358,657; 6,359,105; and 6,593,053. In embodiments, suitable unsaturated polyester base resins may be prepared from diacids and/or anhydrides such as, for example, maleic anhydride, fumaric acid, and the like, and combinations thereof, and diols such as, for example, propoxylated bisphenol A, propylene glycol, and the like, and combinations thereof. In embodiments, a suitable polyester is poly(propoxylated bisphenol A fumarate).

In embodiments, the high molecular weight branched or cross-linked polyester resin has a Mw of greater than about 15,000, in embodiments from about 15,000 to about 1,000,000, in other embodiments from about 20,000 to about 100,000, and a polydispersity index (Mw/Mn) of greater than about 4, in embodiments from about 4 to about 100, in other embodiments from about 6 to about 50, as measured by GPC versus standard polystyrene reference resins.

In embodiments, a cross-linked branched polyester may be utilized as a high molecular weight resin. Such polyester resins may be formed from at least two pre-gel compositions including at least one polyol having two or more hydroxyl groups or esters thereof, at least one aliphatic or aromatic polyfunctional acid or ester thereof, or a mixture thereof having at least three functional groups; and optionally at least one long chain aliphatic carboxylic acid or ester thereof, or aromatic monocarboxylic acid or ester thereof, or mixtures thereof. The two components may be reacted to substantial completion in separate reactors to produce, in a first reactor, a first composition including a pre-gel having carboxyl end groups, and in a second reactor, a second composition including a pre-gel having hydroxyl end groups. The two compositions may then be mixed to create a cross-linked branched polyester high molecular weight resin. Examples of such polyesters and methods for their synthesis include those disclosed in U.S. Patent No. 6,592,913.

In embodiments, branched polyesters may include those resulting from the reaction of dimethylterephthalate, 1,3-butanediol, 1,2-propanediol, and pentaerythritol.

Suitable polyols may contain from about 2 to about 100 carbon atoms and have at least two or more hydroxy groups, or esters thereof. Polyols may include glycerol, pentaerythritol, polyglycol, polyglycerol, and the like, or mixtures thereof. The polyol may include a glycerol. Suitable esters of glycerol include glycerol palmitate, glycerol sebacate, glycerol adipate, triacetin tripropionin, and the like. The polyol may be present in an amount of from about 20% to about 30% weight of the reaction mixture, in embodiments, from about 20% to about 26% weight of the reaction mixture.

Aliphatic polyfunctional acids having at least two functional groups may include saturated and unsaturated acids containing from about 2 to about 100 carbon atoms, or esters thereof, in some embodiments, from about 4 to about 20 carbon atoms. Other aliphatic polyfunctional acids include malonic, succinic, tartaric, malic, citric, fumaric, glutaric, adipic, pimelic, sebacic, suberic, azelaic, sebacic, and the like, or mixtures thereof. Other aliphatic polyfunctional acids which may be utilized include dicarboxylic acids containing a C₃ to C₆ cyclic structure and positional isomers thereof, and include cyclohexane dicarboxylic acid, cyclobutane dicarboxylic acid or cyclopropane dicarboxylic acid.

Aromatic polyfunctional acids having at least two functional groups which may be utilized include terephthalic, isophthalic, trimellitic, pyromellitic and naphthalene 1,4-, 2,3-, and 2,6- dicarboxylic acids.

The aliphatic polyfunctional acid or aromatic polyfunctional acid may be present in an amount of from about 40% to about 65% weight of the reaction mixture, in embodiments, from about 44% to about 60% weight of the reaction mixture.

Long chain aliphatic carboxylic acids or aromatic monocarboxylic acids may include those containing from about 12 to about 26 carbon atoms, or esters thereof, in embodiments, from about 14 to about 18 carbon atoms. Long chain aliphatic carboxylic acids may be saturated or unsaturated. Suitable saturated long chain aliphatic carboxylic acids may include lauric, myristic, palmitic, stearic, arachidic, cerotic, and the like, or combinations thereof. Suitable unsaturated long chain aliphatic carboxylic acids may include dodecylenic, palmitoleic, oleic, linoleic, linolenic, erucic, and the like, or combinations thereof. Aromatic monocarboxylic acids may include benzoic, naphthoic, and substituted napthoic acids. Suitable substituted naphthoic acids may include naphthoic acids substituted with linear or branched alkyl groups containing from about 1 to about 6 carbon atoms such as 1-methyl-2 naphthoic acid and/or 2-isopropyl-1-naphthoic acid. The long chain aliphatic carboxylic acid or aromatic monocarboxylic acids may be present in an amount of from about 0% to about 70% weight of the reaction mixture, in embodiments, of from about 15% to about 30% weight of the reaction mixture.

Additional polyols, ionic species, oligomers, or derivatives thereof, may be used if desired. These additional glycols or polyols may be present in amounts of from about 0% to about 50% weight percent of the reaction mixture. Additional polyols or their derivatives thereof may include propylene glycol, 1,3-butanediol, 1,3-propanediol, 1,4-butanediol, 1,6-hexanediol diethylene glycol, 1,4-cyclohexanediol, 1,4-cyclohexanedimethanol, neopentyl glycol, triacetin, trimethylolpropane, pentaerythritol, cellulose ethers, cellulose esters, such as cellulose acetate, sucrose acetate iso-butyrate and the like.

The amount of high molecular weight resin in a toner particle of the present disclosure, whether in the core, the shell, or both, may be from about 1% to about 30% by weight of the toner, in embodiments from about 2.5% to about 20% by weight, or from about 5% to about 10% by weight of the toner.

In embodiments, the high molecular weight resin, for example a branched polyester, may be present on the surface of toner particles of the present disclosure. The high molecular weight resin on the surface of the toner particles may also be particulate in nature, with high molecular weight resin particles having a diameter of from about 100 nanometers to about 300 nanometers, in embodiments from about 110 nanometers to about 150 nanometers. The high molecular weight resin particles may cover from about 10% to about 90% of the toner surface, in embodiments from about 20 % to about 50 % of the toner surface.

Toner

The resin described above may be utilized to form toner compositions. Such toner compositions may include optional colorants, optional waxes in addition to the at least one ester wax, and other additives. Toners may be formed utilizing any method within the purview of those skilled in the art.

Surfactants

In embodiments, colorants, waxes, and other additives utilized to form toner compositions may be in dispersions including surfactants. Moreover, toner particles may be formed by emulsion aggregation methods where the resin and other components of the toner are placed in one or more surfactants, an emulsion is formed, toner particles are aggregated, coalesced, optionally washed and dried, and recovered.

One, two, or more surfactants may be utilized. The surfactants may be selected from ionic surfactants and nonionic surfactants. Anionic surfactants and cationic surfactants are encompassed by the term "ionic surfactants." In embodiments, the surfactant may be utilized so that it is present in an amount of from about 0.01% to about 5% by weight of the toner composition, for example from about 0.75% to about 4% by weight of the toner composition, in embodiments from about 1% to about 3% by weight of the toner composition.

Examples of nonionic surfactants that can be utilized include, for example, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy) ethanol, available from Rhone-Poulenc as IGEPAL CA-210™, IGEPAL CA-520™, IGEPAL CA-720™, IGEPAL CO-890™, IGEPAL CO-720™, IGEPAL CO-290™, IGEPAL CA-210™, ANTAROX 890™ and ANTAROX 897™. Other examples of suitable nonionic surfactants include a block copolymer of polyethylene oxide and polypropylene oxide, including those commercially available as SYNPERONIC PE/F, in embodiments SYNPERONIC PE/F 108.

Anionic surfactants which may be utilized include sulfates and sulfonates, sodium dodecylsulfate (SDS), sodium dodecylbenzene sulfonate, sodium dodecylnaphthalene sulfate, dialkyl benzenealkyl sulfates and sulfonates, and acids such as abitic acid, which may be obtained from Aldrich, or NEOGEN R™, NEOGEN SC™, NEOGEN RK™ which may be obtained from Daiichi Kogyo Seiyaku, combinations thereof, and the like. Other suitable anionic surfactants include, in embodiments, DOWFAX™ 2A1, an alkyldiphenyloxide disulfonate from The Dow Chemical Company, and/or TAYCA POWER BN2060 from Tayca Corporation (Japan), which are branched sodium dodecyl benzene sulfonates. Combinations of these surfactants and any of the foregoing anionic surfactants may be utilized in embodiments.

Examples of the cationic surfactants, which are usually positively charged, include, for example, alkylbenzyl dimethyl ammonium chloride, dialkyl benzenealkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C12, C15, C17 trimethyl ammonium bromides, halide salts of quaternized polyoxyethylalkylamines, dodecylbenzyl triethyl ammonium chloride, MIRAPOL™ and ALKAQUAT™, available from Alkaril Chemical Company, SANIZOL™ (benzalkonium chloride), available from Kao Chemicals, and the like, and mixtures thereof.

Colorants

As the colorant to be added, various known suitable colorants, such as dyes, pigments, mixtures of dyes, mixtures of pigments, mixtures of dyes and pigments, and the like, may be included in the toner. The colorant may be included in the toner in an amount of, for example, about 0.1 to about 35 percent by weight of the toner, or from about 1 to about 15 weight percent of the toner, or from about 3 to about 10 percent by weight of the toner.

As examples of suitable colorants, mention may be made of carbon black like REGAL 330^{®}; magnetites, such as Mobay magnetites MO8029™ MO8060™; Columbian magnetites; MAPICO BLACKS™ and surface treated magnetites; Pfizer magnetites CB4799™, CB5300™, CB5600™, MCX6369™; Bayer magnetites, BAYFERROX 8600™, 8610™; Northern Pigments magnetites, NP-604™, NP-608™; Magnox magnetites TMB-100™, or TMB-104™; and the like. As colored pigments, there can be selected cyan, magenta, yellow, red, green, brown, blue or mixtures thereof. Generally, cyan, magenta, or yellow pigments or dyes, or mixtures thereof, are used. The pigment or pigments are generally used as water based pigment dispersions.

Specific examples of pigments include SUNSPERSE 6000, FLEXIVERSE and AQUATONE water based pigment dispersions from SUN Chemicals, HELIOGEN BLUE L6900™, D6840™, D7080™, D7020™, PYLAM OIL BLUE™, PYLAM OIL YELLOW™, PIGMENT BLUE 1™ available from Paul Uhlich & Company, Inc., PIGMENT VIOLET 1™, PIGMENT RED 48™, LEMON CHROME YELLOW DCC 1026™, E.D. TOLUIDINE RED™ and BON RED C™ available from Dominion Color Corporation, Ltd., Toronto, Ontario, NOVAPERM YELLOW FGL™, HOSTAPERM PINK E™ from Hoechst, and CINQUASIA MAGENTA™ available from E.I. DuPont de Nemours & Company, and the like. Generally, colorants that can be selected are black, cyan, magenta, or yellow, and mixtures thereof. Examples of magentas are 2,9-dimethyl-substituted quinacridone and anthraquinone dye identified in the Color Index as CI 60710, CI Dispersed Red 15, diazo dye identified in the Color Index as CI 26050, CI Solvent Red 19, and the like. Illustrative examples of cyans include copper tetra(octadecyl sulfonamido) phthalocyanine, x-copper phthalocyanine pigment listed in the Color Index as CI 74160, CI Pigment Blue, Pigment Blue 15:3, and Anthrathrene Blue, identified in the Color Index as CI 69810, Special Blue X-2137, and the like. Illustrative examples of yellows are diarylide yellow 3,3-dichlorobenzidene acetoacetanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33 2,5-dimethoxy-4-sulfonanilide phenylazo-4'-chloro-2,5-dimethoxy acetoacetanilide, and Permanent Yellow FGL. Colored magnetites, such as mixtures of MAPICO BLACK™, and cyan components may also be selected as colorants. Other known colorants can be selected, such as Levanyl Black A-SF (Miles, Bayer) and Sunsperse Carbon Black LHD 9303 (Sun Chemicals), and colored dyes such as Neopen Blue (BASF), Sudan Blue OS (BASF), PV Fast Blue B2G01 (American Hoechst), Sunsperse Blue BHD 6000 (Sun Chemicals), Irgalite Blue BCA (Ciba-Geigy), Paliogen Blue 6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange 220 (BASF), Paliogen Orange 3040 (BASF), Ortho Orange OR 2673 (Paul Uhlich), Paliogen Yellow 152, 1560 (BASF), Lithol Fast Yellow 0991K (BASF), Paliotol Yellow 1840 (BASF), Neopen Yellow (BASF), Novoperm Yellow FG 1 (Hoechst), Permanent Yellow YE 0305 (Paul Uhlich), Lumogen Yellow D0790 (BASF), Sunsperse Yellow YHD 6001 (Sun Chemicals), Suco-Gelb L1250 (BASF), Suco-Yellow D1355 (BASF), Hostaperm Pink E (American Hoechst), Fanal Pink D4830 (BASF), Cinquasia Magenta (DuPont), Lithol Scarlet D3700 (BASF), Toluidine Red (Aldrich), Scarlet for Thermoplast NSD PS PA (Ugine Kuhlmann of Canada), E.D. Toluidine Red (Aldrich), Lithol Rubine Toner (Paul Uhlich), Lithol Scarlet 4440 (BASF), Bon Red C (Dominion Color Company), Royal Brilliant Red RD-8192 (Paul Uhlich), Oracet Pink RF (Ciba-Geigy), Paliogen Red 3871K (BASF), Paliogen Red 3340 (BASF), Lithol Fast Scarlet L4300 (BASF), combinations of the foregoing, and the like.

Wax

In embodiments, the toner particles include an ester wax that is compatible with the toner resin components. In embodiments, the toner particles include an ester wax that is compatible with the toner amorphous resin components. Typical waxes that may be selected include waxes having, for example, a weight average molecular weight of from about 500 to about 20,000, in embodiments from about 1,000 to about 10,000.

In embodiments, an ester wax is selected wherein the Delta Solubility Parameter (ΔSP) between the amorphous polyester and the ester wax is from about 0.1 to about 1.7, or from about 0.5 to about 1.4. As a result, the surface of the toner may possess higher elasticity and may result in preferred toner performance such as a reduction in additive impaction, improved toner flow during xerographic use and a reduced tendency for toner blocking during transportation and storage, particularly under high temperature and high humidity conditions. Further, as a result, the toner may provide excellent fusing performance in an oil-less or low oil fuser.

As used herein, an SP value (solubility parameter) means a value obtained by the Fedors method. The SP value may be defined by the following equation: $SP = \sqrt{\frac{Δ ⁢ E}{V}} = \sqrt{\frac{{\sum }_{i} Δ ei}{{\sum }_{i} Δ vi}}$

In the equation, SP represents a solubility parameter, ΔE represents a cohesive energy (cal/mol), V represents mole volume (cm³/mol), Δei represents a vaporization energy of an i^{th} atom or atomic moiety (cal/atom or atomic moiety), Δvi represents a mole volume of an i^{th} atom or atomic moiety (cm³/atom or atomic moiety), and i represents an integer of 1 or more.

The SP value represented by the above equation may be obtained so that its unit becomes cal^{1/2}/cm^{3/2} as a custom, and is expressed dimensionlessly. In addition, since a relative difference in the SP value (ΔSP) between a high molecular weight resin and the linear resin utilized in the formation of a toner is meaningful, the difference in the SP values, ΔSP, is also expressed dimensionlessly.

In embodiments, the ester wax may be present in an amount of from about 1 weight percent to about 15 weight percent based upon the total weight of the toner, although not limited.

Ester waxes are ester compounds derived from the combination of a carboxylic acid and alcohol components. The carboxylic acid typically is a single type of saturated linear monocarboxylic acid having 10 to 40 carbon atoms. The alcohol typically is a single kind of saturated linear monohydric alcohol having 10 to 30 carbon atoms or a single kind of polyhydric alcohol having 2 to 6 hydroxyl groups and having 2 to 30 carbon atoms. Ester waxes that may be selected include monoester, diester, trimester, and higher ester waxes such as ester waxes obtained from higher fatty acids and higher alcohols, wherein higher means having 6 or more carbons, ester waxes obtained from higher fatty acids and monovalent or multivalent lower alcohols, ester waxes obtained from higher fatty acid and multivalent alcohol multimers, sorbitan higher fatty acid ester waxes, cholesterol higher fatty acid ester waxes, plant-based ester waxes, such as carnauba wax, rice bran wax, candelilla wax, sumac wax, and jojoba oil, animal-based ester waxes, such as beeswax, mineral-based ester waxes, such as montan wax, acid modified polyethylene waxes, and mixtures and combinations thereof. Higher fatty acids and higher alcohols are typically considered to be any acid or alcohol with greater than six total carbons.

Specific examples of suitable ester waxes include butyl stearate, stearyl stearate, propyl oleate, hexadecyl myristate, arachidyl arachidate, behenyl behenate, glyceride monostearate, glyceride distearate, pentaerythritol tetrabehenate, diethyleneglycol monostearate, dipropyleneglycol distearate, diglyceryl distearate, triglyceryl tetrastearate, sorbitan monostearate, cholesteryl stearate, and mixtures and combinations thereof. In embodiments, a selected ester wax is behenyl behenate of the formula CH₃(CH₂)₂₀CO₂-(CH₂)₂₁CH₃, for example, Esprix^{®} N-252 available from Esprix^{®} Technologies.

Toner Preparation

The toner particles may be prepared by any method within the purview of one skilled in the art. Although embodiments relating to toner particle production are described below with respect to emulsion-aggregation processes, any suitable method of preparing toner particles may be used, including chemical processes, such as suspension and encapsulation processes disclosed in U.S. Patent Nos. 5,290,654 and 5,302,486. In embodiments, toner compositions and toner particles may be prepared by aggregation and coalescence processes in which small-size resin particles are aggregated to the appropriate toner particle size and then coalesced to achieve the final toner-particle shape and morphology.

In embodiments, toner compositions may be prepared by emulsion-aggregation processes, such as a process that includes aggregating a mixture of an optional colorant, and any other desired or required additives, and emulsions including the resins and/or high molecular weight and cross-linked resins and ester waxes described above, optionally in surfactants as described above, and then coalescing the aggregate mixture. A mixture may be prepared by adding a colorant, an ester wax, and optionally other materials, which may also be optionally in a dispersion(s) including a surfactant, to the emulsion, which may be a mixture of two or more emulsions containing the resin. The pH of the resulting mixture may be adjusted by an acid such as, for example, acetic acid, nitric acid or the like. In embodiments, the pH of the mixture may be adjusted to from about 2 to about 5. Additionally, in embodiments, the mixture may be homogenized. If the mixture is homogenized, homogenization may be accomplished by mixing at about 600 to about 6,000 revolutions per minute. Homogenization may be accomplished by any suitable means, including, for example, an IKA ULTRA TURRAX® T50 probe homogenizer.

Following the preparation of the above mixture, an aggregating agent may be added to the mixture. Any suitable aggregating agent may be utilized to form a toner. Suitable aggregating agents include, for example, aqueous solutions of a divalent cation or a multivalent cation material. The aggregating agent may be, for example, polyaluminum halides such as polyaluminum chloride (PAC), or the corresponding bromide, fluoride, or iodide, polyaluminum silicates such as polyaluminum sulfosilicate (PASS), and water soluble metal salts including aluminum chloride, aluminum nitrite, aluminum sulfate, potassium aluminum sulfate, calcium acetate, calcium chloride, calcium nitrite, calcium oxylate, calcium sulfate, magnesium acetate, magnesium nitrate, magnesium sulfate, zinc acetate, zinc nitrate, zinc sulfate, zinc chloride, zinc bromide, magnesium bromide, copper chloride, copper sulfate, and combinations thereof. In embodiments, the aggregating agent may be added to the mixture at a temperature that is below the glass transition temperature (Tg) of the resin.

The aggregating agent may be added to the mixture utilized to form a toner in an amount of, for example, from about 0.1% to about 10% by weight, in embodiments from about 0.2% to about 8% by weight, in other embodiments from about 0.5% to about 5% by weight, of the resin in the mixture. This should provide a sufficient amount of agent for aggregation.

The particles may be permitted to aggregate until a predetermined desired particle size is obtained. A predetermined desired size refers to the desired particle size to be obtained as determined prior to formation, and the particle size being monitored during the growth process until such particle size is reached. Samples may be taken during the growth process and analyzed, for example with a Coulter Counter, for average particle size. The aggregation thus may proceed by maintaining the elevated temperature, or slowly raising the temperature to, for example, from about 40°C to about 100°C, and holding the mixture at this temperature for a time of from about 0.5 hours to about 6 hours, in embodiments from about hour 1 to about 5 hours, while maintaining stirring, to provide the aggregated particles. Once the predetermined desired particle size is reached, then the growth process is halted.

The growth and shaping of the particles following addition of the aggregation agent may be accomplished under any suitable conditions. For example, the growth and shaping may be conducted under conditions in which aggregation occurs separate from coalescence. For separate aggregation and coalescence stages, the aggregation process may be conducted under shearing conditions at an elevated temperature, for example of from about 40°C to about 90°C, in embodiments from about 45°C to about 80°C, which may be below the glass transition temperature of the resin as discussed above.

Once the desired final size of the toner particles is achieved, the pH of the mixture may be adjusted with a base to a value of from about 3 to about 10, and in embodiments from about 5 to about 9. The adjustment of the pH may be utilized to freeze, that is to stop, toner growth. The base utilized to stop toner growth may include any suitable base such as, for example, alkali metal hydroxides such as, for example, sodium hydroxide, potassium hydroxide, ammonium hydroxide, combinations thereof, and the like. In embodiments, ethylene diamine tetraacetic acid (EDTA) may be added to help adjust the pH to the desired values noted above.

Shell Resin

In embodiments, after aggregation, but prior to coalescence, a resin coating may be applied to the aggregated particles to form a shell thereover. Any resin described above as suitable for forming the core resin may be utilized as the shell. In embodiments, a high molecular weight resin latex as described above may be included in the shell. In yet other embodiments, the high molecular weight resin latex described above may be combined with a resin that may be utilized to form the core, and then added to the particles as a resin coating to form a shell.

In embodiments, resins which may be utilized to form a shell include, but are not limited to, a high molecular weight resin latex described above, and/or the amorphous resins described above for use as the core. In embodiments, an amorphous resin which may be utilized to form a shell in accordance with the present disclosure includes an amorphous polyester, optionally in combination with a high molecular weight resin latex described above. For example, in embodiments, an amorphous resin of formula I above may be combined with a cross-linked styrene-n-butyl acrylate resin to form a high molecular weight resin shell. Multiple resins may be utilized in any suitable amounts. In embodiments, a first amorphous polyester resin, for example an amorphous resin of formula I above, may be present in an amount of from about 20 percent by weight to about 100 percent by weight of the total shell resin, in embodiments from about 30 percent by weight to about 90 percent by weight of the total shell resin. Thus, in embodiments, a second resin may be present in the shell resin in an amount of from about 0 percent by weight to about 80 percent by weight of the total shell resin, in embodiments from about 10 percent by weight to about 70 percent by weight of the shell resin.

The shell resin may be applied to the aggregated particles by any method within the purview of those skilled in the art. In embodiments, the resins utilized to form the shell may be in an emulsion including any surfactant described above. The emulsion possessing the resins, optionally the high molecular weight resin latex described above, may be combined with the aggregated particles described above so that the shell forms over the aggregated particles.

The formation of the shell over the aggregated particles may occur while heating to a temperature of from about 30°C to about 80°C, in embodiments from about 35°C to about 70°C. The formation of the shell may take place for a period of time of from about 5 minutes to about 10 hours, in embodiments from about 10 minutes to about 5 hours.

Coalescence

Following aggregation to the desired particle size and application of any optional shell, the particles may then be coalesced to the desired final shape, the coalescence being achieved by, for example, heating the mixture to a temperature of from about 45°C to about 100°C, in embodiments from about 55°C to about 99°C, which may be at or above the glass transition temperature of the resins utilized to form the toner particles, and/or reducing the stirring, for example to from about 100 rpm to about 1,000 rpm, in embodiments from about 200 rpm to about 800 rpm. Higher or lower temperatures may be used, it being understood that the temperature is a function of the resins used for the binder. Coalescence may be accomplished over a period of from about 0.01 to about 9 hours, in embodiments from about 0.1 to about 4 hours.

After aggregation and/or coalescence, the mixture may be cooled to room temperature, such as from about 20°C to about 25°C. The cooling may be rapid or slow, as desired. A suitable cooling method may include introducing cold water to a jacket around the reactor. After cooling, the toner particles may be optionally washed with water, and then dried. Drying may be accomplished by any suitable method for drying including, for example, freeze-drying.

Where the core, the shell, or both includes a branched high molecular weight resin as described above, the presence of the high molecular weight resin may prevent the crystalline resin in the core from migrating to the toner surface. This may especially occur where the high molecular weight resin is present in the shell. In addition, the shell resin(s) may be less compatible with the crystalline resin utilized in forming the core, which may result in a higher toner glass transition temperature (Tg), and thus improved blocking and charging characteristics may be obtained, including A-zone charging. In addition, the high molecular weight resin utilized in the formation of a core-shell particle may have a high viscosity of greater than about 10,000,000 Poise, in embodiments greater than about 50,000,000 Poise, which may be able to prevent any crystalline resin in the core from migrating to the toner surface and thus improve A-zone charging. Moreover, toners of the present disclosure having a high molecular weight resin latex in the core and/or shell may exhibit excellent document offset performance characteristics, as well as reduced peak gloss, in embodiments from about 5 Gardner gloss units (ggu) to about 100 ggu, in other embodiments from about 10 ggu to about 80 ggu, which may be desirable for reproduction of text and images, as some users object to high gloss and the differential which may occur between low gloss and high gloss.

In embodiments, the high molecular weight resin utilized in forming the core and/or shell may be present in an amount of from about 2 percent by weight to about 30 percent by weight of the dry toner particles, in embodiments from about 5 percent by weight to about 25 percent by weight of the dry toner particles.

Toner particles possessing a core and or shell possessing a high molecular weight resin as described above may, in embodiments, have a glass transition temperature of from about 30°C to about 80°C, in embodiments from about 35°C to about 70°C.

Additives

In embodiments, the toner particles may also contain other optional additives, as desired or required. For example, the toner may include positive or negative charge control agents, for example in an amount of from about 0.1 to about 10 percent by weight of the toner, in embodiments from about 1 to about 3 percent by weight of the toner. Examples of suitable charge control agents include quaternary ammonium compounds inclusive of alkyl pyridinium halides; bisulfates; alkyl pyridinium compounds, including those disclosed in U.S. Patent No. 4,298,672; organic sulfate and sulfonate compositions, including those disclosed in U.S. Patent No. 4,338,390; cetyl pyridinium tetrafluoroborates; distearyl dimethyl ammonium methyl sulfate; aluminum salts such as BONTRON E84™ or E88™ (Hodogaya Chemical); combinations thereof, and the like. Such charge control agents may be applied simultaneously with the shell resin described above or after application of the shell resin.

There can also be blended with the toner particles external additive particles including flow aid additives, which additives may be present on the surface of the toner particles. Examples of these additives include metal oxides such as titanium oxide, silicon oxide, tin oxide, mixtures thereof, and the like; colloidal and amorphous silicas, such as AEROSIL®, metal salts and metal salts of fatty acids inclusive of zinc stearate, aluminum oxides, cerium oxides, and mixtures thereof. Each of these external additives may be present in an amount of from about 0.1 percent by weight to about 5 percent by weight of the toner, in embodiments of from about 0.25 percent by weight to about 3 percent by weight of the toner. Suitable additives include those disclosed in U.S. Patent Nos. 3,590,000, 3,800,588, and 6,214,507. Again, these additives may be applied simultaneously with the shell resin described above or after application of the shell resin.

In other embodiments, a "sol-gel" metal oxide may be used as the high molecular weight resin in accordance with the present disclosure. The sol-gel metal oxide may be produced by a sol-gel process, as compared to one produced by other well-known processes, such as fuming. It has been found that the sol-gel process imparts different properties to the resultant metal oxide product. For example, metal oxides formed by a sol-gel process have been found to be more spherical than metal oxides formed by other processes. Thus, for example, a sol-gel silica may be a silica synthesized by the controlled hydrolysis and condensation of tetraethoxysilane or other suitable starting materials. The sol-gel process may be carried out in alcohol solvents with added homopolymer solutes to control the structure of the precipitated silicon dioxide product.

Any suitable sol-gel metal oxide base material can be used. Suitable metal oxides include, but are not limited to, silica, titania, ceria, zirconia, alumina, mixtures thereof, and the like. For example, suitable sol-gel metal oxide products include KEP-10 and KEP-30, both of which are sol-gel silicas available from ESPRIX^{®}, Inc. and X24 available from Shin-Etsu Chemical Co.

In embodiments, the sol-gel metal oxide may have a primary particle size of from about 100 nanometers to about 600 nanometers. Because the sol-gel metal oxides typically disperse as primary particles, the penchant for inter-particle cohesion via chain entanglements is minimized. However, in embodiments sol-gel metal oxide materials having sizes outside of these ranges can be used.

In embodiments, toners of the present disclosure may be utilized as ultra low melt (ULM) toners. In embodiments, the dry toner particles having a core and/or shell including the high molecular weight resin of the present disclosure may, exclusive of external surface additives, have the following characteristics:

(1) Volume average diameter (also referred to as "volume average particle diameter") of from about 3 to about 25 micrometers (µm), in embodiments from about 4 to about 15 µm, in other embodiments from about 5 to about 12 µm.

(2) Number Average Geometric Size Distribution (GSDn) and/or Volume Average Geometric Size Distribution (GSDv) of from about 1.05 to about 1.55, in embodiments from about 1.1 to about 1.4.

(3) Circularity of from about 0.9 to about 1, in embodiments from about 0.93 to about 0.98 (measured with, for example, a Sysmex FPIA 2100 analyzer).

The characteristics of the toner particles may be determined by any suitable technique and apparatus. Volume average particle diameter D₅₀ᵥ, GSDv, and GSDn may be measured by means of a measuring instrument such as a Beckman Coulter Multisizer 3, operated in accordance with the manufacturer's instructions. Representative sampling may occur as follows: a small amount of toner sample, about 1 gram, may be obtained and filtered through a 25 micrometer screen, then put in isotonic solution to obtain a concentration of about 10%, with the sample then run in a Beckman Coulter Multisizer 3.

Toners produced in accordance with the present disclosure may possess excellent charging characteristics when exposed to extreme relative humidity (RH) conditions. The low-humidity zone (C-zone) may be about 10°C/15% RH, while the high humidity zone (A-zone) may be about 28°C/85% RH. Toners of the present disclosure may possess a parent toner charge per mass ratio (Q/M) in ambient conditions (B-zone) of about 21°C/50% RH of from about -3 µC/g to about -50 µC/g, in embodiments from about -5 µC/g to about -40 µC/g, and a final toner charging after surface additive blending of from - 10 µC/g to about -50 µC/g, in embodiments from about -20 µC/g to about -40 µC/g.

Developers

The toner particles may be formulated into a developer composition. The toner particles may be mixed with carrier particles to achieve a two-component developer composition. The toner concentration in the developer may be from about 1% to about 25% by weight of the total weight of the developer, in embodiments from about 2% to about 15% by weight of the total weight of the developer.

Carriers

Examples of carrier particles that can be utilized for mixing with the toner include those particles that are capable of triboelectrically obtaining a charge of opposite polarity to that of the toner particles. Illustrative examples of suitable carrier particles include granular zircon, granular silicon, glass, steel, nickel, ferrites, iron ferrites, silicon dioxide, and the like. Other carriers include those disclosed in U.S. Patent Nos. 3,847,604, 4,937,166, and 4,935,326.

The selected carrier particles can be used with or without a coating. In embodiments, the carrier particles may include a core with a coating thereover which may be formed from a mixture of polymers that are not in close proximity thereto in the triboelectric series. The coating may include fluoropolymers, such as polyvinylidene fluoride resins, terpolymers of styrene, methyl methacrylate, and/or silanes, such as triethoxy silane, tetrafluoroethylenes, other known coatings and the like. For example, coatings containing polyvinylidenefluoride, available, for example, as KYNAR 301F™, and/or polymethylmethacrylate, for example having a weight average molecular weight of about 300,000 to about 350,000, such as commercially available from Soken, may be used. In embodiments, polyvinylidenefluoride and polymethylmethacrylate (PMMA) may be mixed in proportions of from about 30 to about 70 weight % to about 70 to about 30 weight %, in embodiments from about 40 to about 60 weight % to about 60 to about 40 weight %. The coating may have a coating weight of, for example, from about 0.1 to about 5% by weight of the carrier, in embodiments from about 0.5 to about 2% by weight of the carrier.

In embodiments, PMMA may optionally be copolymerized with any desired comonomer, so long as the resulting copolymer retains a suitable particle size. Suitable comonomers can include monoalkyl, or dialkyl amines, such as a dimethylaminoethyl methacrylate, diethylaminoethyl methacrylate, diisopropylaminoethyl methacrylate, or t-butylaminoethyl methacrylate, and the like. The carrier particles may be prepared by mixing the carrier core with polymer in an amount from about 0.05 to about 10 percent by weight, in embodiments from about 0.01 percent to about 3 percent by weight, based on the weight of the coated carrier particles, until adherence thereof to the carrier core by mechanical impaction and/or electrostatic attraction.

Various effective suitable means can be used to apply the polymer to the surface of the carrier core particles, for example, cascade roll mixing, tumbling, milling, shaking, electrostatic powder cloud spraying, fluidized bed, electrostatic disc processing, electrostatic curtain, combinations thereof, and the like. The mixture of carrier core particles and polymer may then be heated to enable the polymer to melt and fuse to the carrier core particles. The coated carrier particles may then be cooled and thereafter classified to a desired particle size.

In embodiments, suitable carriers may include a steel core, for example of from about 25 to about 100 µm in size, in embodiments from about 50 to about 75 µm in size, coated with about 0.5% to about 10% by weight, in embodiments from about 0.7% to about 5% by weight, of a conductive polymer mixture including, for example, methylacrylate and carbon black using the process described in U.S. Patent Nos. 5,236,629 and 5,330,874.

The carrier particles can be mixed with the toner particles in various suitable combinations. The concentrations are may be from about 1% to about 20% by weight of the toner composition. However, different toner and carrier percentages may be used to achieve a developer composition with desired characteristics.

Imaging

The toners can be utilized for electrostatographic or xerographic processes, including those disclosed in U.S. Patent No. 4,295,990. In embodiments, any known type of image development system may be used in an image developing device, including, for example, magnetic brush development, jumping single-component development, hybrid scavengeless development (HSD), and the like. These and similar development systems are within the purview of those skilled in the art.

Imaging processes include, for example, preparing an image with a xerographic device including a charging component, an imaging component, a photoconductive component, a developing component, a transfer component, and a fusing component. In embodiments, the development component may include a developer prepared by mixing a carrier with a toner composition described herein. The xerographic device may include a high speed printer, a black and white high speed printer, a color printer, and the like.

Once the image is formed with toners/developers via a suitable image development method such as any one of the aforementioned methods, the image may then be transferred to an image receiving medium such as paper and the like. In embodiments, the toners may be used in developing an image in an image-developing device utilizing a fuser roll member. Fuser roll members are contact fusing devices that are within the purview of those skilled in the art, in which heat and pressure from the roll may be used to fuse the toner to the image-receiving medium. In embodiments, the fuser member may be heated to a temperature above the fusing temperature of the toner, for example to temperatures of from about 70°C to about 160°C, in embodiments from about 80°C to about 150°C, in other embodiments from about 90°C to about 140°C, after or during melting onto the image receiving substrate.

.

### EXAMPLES

The following Examples are being submitted to further define various species of the present disclosure. These Examples are intended to be illustrative only and are not intended to limit the scope of the present disclosure. Also, parts and percentages are by weight unless otherwise indicated. As used herein, "room temperature" refers to a temperature of from about 20 °C to about 25° C.

Solubility parameters were calculated as described by Fedors (Polymer Engineering and Science, February, 1974, Volume 14, No. 2, pages 147-154 and Polymer Engineering and Science, February, 1974, Volume 14, No. 6, page 472). Polymer molecular weights were determined by gel permeation chromatography (GPC) of the chloroform soluble fraction (0.2 micron filter) on an instrument available from Shimadzu Scientific Instruments Corporation using 2 PL Mixed-C columns available from Polymer Laboratories (Varian, Inc.) against polystyrene standards that ranged from 590 to 841,700 g/mol. Values for Mₙ, Mₚ and M_{w} were calculated automatically by software available from Polymer Laboratories.

### Comparative Example 1

Toner-1 (Comparative Toner, No Wax). About 397.99 grams of a linear amorphous resin in an emulsion (about 17.03 weight % resin) was added to a 2 liter beaker. The linear amorphous resin was of the following formula:

wherein m was from about 5 to about 1000 and was produced following the procedures described in U.S. Patent No. 6,063,827. About 74.27 grams of an unsaturated crystalline polyester ("UCPE") resin including ethylene glycol and a mixture of dodecanedioic acid and fumaric acid co-monomers of the following formula:

wherein b was from 5 to 2000 and d was from 5 to 2000 in an emulsion (about 19.98 weight % resin), synthesized following the procedures described in Example 2 of U.S. Patent Application Publication No. 2008/0107990, about 29.24 grams of a cyan pigment, Pigment Blue 15:3, (about 17 weight %), and about 281.8 grams of deionized water were added to the beaker. About 36 grams of Al₂(SO₄)₃ (about 1 weight %) was added as a flocculent under homogenization by mixing the mixture at about 3000 to 4000 rpm. The mixture was subsequently transferred to a 2 liter Buchi reactor, and heated to about 45.9°C for aggregation and mixed at a speed of about 750 rpm. The particle size was monitored with a Coulter Counter until the size of the particles reached an average volume particle size of about 6.83 µm with a Geometric Size Distribution ("GSD") of about 1.21. About 198.29 grams of the above emulsion with the resin of Formula I was then added to the particles to form a shell thereover, resulting in particles possessing a core/shell structure with an average particle size of about 8.33 µm, and a GSD of about 1.21. Thereafter, the pH of the reaction slurry was increased to about 6.7 by adding NaOH followed by the addition of about 0.45 pph EDTA (based on dry toner) to freeze, that is stop, the toner growth. After stopping the toner growth, the reaction mixture was heated to about 69° C and kept at that temperature for about 1 hour for coalescence. The resulting toner particles had a final average volume particle size of about 8.07, a GSD of about 1.22, and a circularity of about 0.976. The toner slurry was then cooled to room temperature, separated by sieving (utilizing a 25 µm sieve) and filtered, followed by washing and freeze drying. The parent toner was surface additive blended with small particle, hydrophobically treated fumed silica and titania and zinc stearate as is described in Example 9 of U.S. Patent No. 6,365,316.

### Comparative Example 2

Toner-2 (Comparative Toner made with 9 % polymethylene wax). An emulsion of a Fisher-Tropsch polymethylene wax obtained from IGI, Inc. was prepared via the method described in detail in Example 3.

Into a 2 liter glass reactor equipped with an overhead stirrer and heating mantle was added 136.25 grams linear propoxylated bisphenol A fumarate resin (Formula I) emulsion (48.50 wt %), 54.93 grams unsaturated crystalline polyester resin emulsion (31.52 wt %, UCPE, Formula II), 41.97 grams polymethylene wax (IGI wax emulsion) (30.77 wt %) and 34.11 grams cyan pigment (PB-15:3, Sun Chemical, 17.00 wt %). Al₂(SO₄)₃ (41.82 g, 1 wt %) was added in as flocculent under homogenization. The mixture was subsequently heated to 47.2 °C for aggregation at about 270 rpm. The particle size was monitored with a Coulter Counter until the core particles reached a volume average particle size of 7.42 µm with a GSD of 1.20, and then 80.83 grams of the linear propoxylated bisphenol A fumarate resin emulsion (Formula I, 48.50 wt %) was added as shell, resulting in a core-shell structured particles with an average particle size of 9.25 microns, GSD 1.19. Thereafter, the pH of the reaction slurry was then increased to 6.8 using NaOH to freeze the toner growth. After freezing, the reaction mixture was heated to 69.4 °C, and pH was reduced to 6.15 for coalescence. However, the toner particles started growing and falling apart at the same time with an initial sign of coalescence. About 3 hours later, at 70.7 °C, pH 6.00, toner particles were finally formed; however, attempts to maintain the desired toner particle size and particle size distribution failed. The toner had a final average particle size of 15.76 microns, GSDv of 1.25, and GSDn of 1.94. The difficulty in coalescence step and the inability to freeze the particle size and distribution are believed to be the direct result of incompatibility of the polymethylene wax and the linear amorphous polyester of Formula I. This toner was therefore unsuitable for fusing and xerographic testing.

### Example 3

Preparation of Esprix^{®} N-252 Wax Emulsion. A wax emulsion is prepared by adding 47.09 grams of Esprix^{®} N-252 ester wax into a 2 liter beaker containing about 480 grams of ethyl acetate. The mixture is stirred at about 250 revolutions per minute and heated to about 71°C to dissolve the wax in the ethyl acetate. 2.54g (46.8 wt %) of Dowfax is measured into a 4 liter Pyrex^{®} glass flask reactor containing about 1,000 grams of deionized water and heated to about 70°C. Homogenization of said heated water solution in said 4 liter glass flask reactor is commenced with an IKA Ultra Turrax^{®} T50 homogenizer at 4,000 revolutions per minute. The heated resin solution is then slowly poured into the water solution as the mixture continues to be homogenized, the homogenizer speed is increased to 6,400 revolutions per minute and homogenization is carried out at these conditions for about 30 minutes. Upon completion of homogenization, the glass flask reactor and its contents are placed in a heating mantle and connected to a distillation device. The mixture is stirred at about 300 revolutions per minute and the temperature of said mixture is increased to 80°C at about 1°C per minute to distill off the ethyl acetate from the mixture. Stirring of the said mixture is continued at 80°C for about 120 minutes followed by cooling at about 2°C per minute to room temperature. The product is screened through a 20 micron sieve. The resulting resin emulsion is comprised of about 8.12 per cent by weight solids in water, and has a volume average diameter of about 180.4 nanometers as measured with a HONEYWELL MICROTRAC^{®} UPA150 particle size analyzer.

### Example 4

Toner 3 (5% Esprix® N-252 ester wax). Into a 2 liter beaker was added 304.79 grams linear propoxylated bisphenol A fumarate resin (Formula I) emulsion (20.09 wt %), 40.23 grams unsaturated crystalline polyester resin emulsion (35.48 wt %, UCPE, Formula II), 75.11 grams ester wax (Esprix^{®} N-252 wax emulsion) (8.12 wt %) and 33.76 g cyan pigment (PB 15:3, 14.60 wt %). Al₂(SO₄)₃ (35.54 grams, 1 wt %) was added in as flocculent under homogenization. The mixture was subsequently transferred to a 2 liter Buchi, and heated to 47.4 °C for aggregation at rpm 700 rpm. The particle size was monitored with a Coulter Counter until the core particles reached a volume average particle size of 7.56 µm with a GSD of 1.21, and then 76.69 grams of the linear propoxylated bisphenol A fumarate resin emulsion (Formula I, 43.45 wt %) was added as shell, resulting in a core-shell structured particles with an average particle size of 9.14 microns, GSD 1.21. Thereafter, the pH of the reaction slurry was then increased to 7.5 using NaOH to freeze the toner growth. After freezing, the reaction mixture was heated to 73.3°C, and pH was reduced to 5.95 for coalescence. The toner quenched after coalescence, and it has a final particle size of 8.77 microns, GSD of 1.23, and Circularity of 0.964. The toner slurry was then cooled to room temperature, separated by sieving (25 µm), filtration, followed by washing and freeze dried. The parent toner was surface additive blended with small particle, hydrophobically treated fumed silica and titania and zinc stearate as is described in Example 9 of U.S. Patent No. 6,365,316.

### Example 5

Toner 4 (9% Esprix^{®} N-252 ester wax). Into a 2 liter beaker was added 368.6 grams linear propoxylated bisphenol A fumarate resin emulsion (16.73 wt %), 46.62 grams unsaturated CPE resin emulsion (UCPE, 33.46 wt %, Formula II), 147.69 grams Esprix^{®} N-252 wax emulsion (8.12 wt %) and 36.88 grams cyan pigment (PB15:3, Sun Chemical, 14.60 wt %). Al₂(SO₄)₃ (38.83 grams, 1 wt %) was added in as flocculent under homogenization. The mixture was subsequently transferred to a 2 liter Buchi, and heated to 44.4 °C for aggregation at rpm 700 rpm. The particle size was monitored with a Coulter Counter until the core particles reached a volume average particle size of 7.34 µm with a GSD of 1.22, and then 218.66 grams of the above linear propoxylated bisphenol A fumarate resin emulsion (Formula I) was added as shell, resulting in a core-shell structured particles with an average particle size of 8.59 microns, GSD 1.21. Thereafter, the pH of the reaction slurry was then increased to 7.5 using NaOH to freeze the toner growth. After freezing, the reaction mixture was heated to 73.2°C, and pH was reduced to 5.99 for coalescence. The toner quenched after coalescence, and it has a final particle size of 8.77 microns, GSD of 1.29, and Circularity of 0.962. The toner slurry was then cooled to room temperature, separated by sieving (25 µm), filtration, followed by washing and freeze dried. The parent toner was surface additive blended with small particle, hydrophobically treated fumed silica and titania and zinc stearate as is described in Example 9 of U.S. Patent No. 6,365,316.

Fusing Performance

Patches of toner at 1.0 mg/cm² laydown were fused onto 90 gsm Xerox^{®} Color Xpressions Plus paper using an oil-less fusing fixture and the resulting fused prints were evaluated for gloss, crease, hot offset and document offset. A summary of toner properties is shown in Table 1 below.

**Table 1**

| | Toner-1 Comparative Example 1 | Toner-2 Comparative Example 2 | Toner-3 Example 4 | Toner-4 Example 5 |
|---|---|---|---|---|
| **% Resin 1** (linear propoxylated bisphenol A fumarate resin) | 84.2% | 75.2% | 79.2% | 75.2% |
| **Resin 1 SP** | 9.91 | 9.91 | 9.91 | 9.91 |
| **% Resin 2** (unsaturated crystalline polyester resin) | 12% | 12% | 12% | 12% |
| **Wax** | None | Polymethylene Wax | N-252 | N-252 |
| **% Wax** | 0% | 9% | 5% | 9% |
| **Wax SP** | NA | 8.07 | 8.59 | 8.59 |
| **Delta SP** | NA | 1.84 | 1.32 | 1.32 |
| **% cyan pigment** | 3.8% | 3.8% | 3.8% | 3.8% |
| **Cold Offset Temperature** | NA | NA | 117 °C | 123 °C |
| **Hot Offset Temperature** | NA | NA | 175 °C | >210 °C |
| **Fusing Latitude** | NA | NA | 57 °C | >79 °C |

| | | | | |
|---|---|---|---|---|
| *SP = Solubility Parameter, NA = not applicable | | | | |

Fusing data for Comparative Toners 1 and 2 could not be obtained as the fusing device did not include fusing oil as a release agent and was designed to fuse wax containing toners only. Attempts to fuse non-wax containing toners would only resulted in paper jams as the paper would not release properly from the fuser roll subsequent to fusing of the toner to the page.

Fusing data show that toners 3 and 4 have very good fusing latitude, low minimum fix temperature, good hot offset temperature characteristics, and acceptable gloss. This indicates that the wax and crystalline polyester were both successfully incorporated into the final particle.

Charging Performance

Charging characteristics were determined by testing developers made by combining about 4.5 grams of toner with about 100 grams of carrier (65 micron steel core, Hoeganaes Corporation) coated with about 1% by weight of polymethylmethacrylate. The developers were placed in a glass jar and mixed using a paint shaker at about 715 cycles per minute under the specified conditions of time, temperature and relative humidity, with A Zone meaning 80° F. and 80 percent relative humidity (RH), and C zone meaning 60° F. and 20 percent RH. The triboelectric (tribo) charge was determined by the conventional tribo blow-off technique. The RH sensitivity was the ratio of the tribo value at 60 deg./ 20 percent RH to the tribo value at 80 deg./ 80 percent RH. A summary of the results is shown in Table 2 below. Charging data for Comparative Toner 2 was not obtained due to the unsuitable nature of the particles that were obtained.

**Table 2**

| | **Toner-1** Comparative Example 1 | **Toner-3** Example 4 | **Toner-4** Example 5 |
|---|---|---|---|
| **5 min A-Zone Tribo** | -3.7 | -4.1 | -2.2 |
| **60 min A-Zone Tribo** | -3.6 | -6.1 | -4.8 |
| **5 min C-Zone Tribo** | -16.6 | -18.4 | -5.1 |
| **60 min C-Zone Tribo** | -13.7 | -18.0 | -10.0 |
| **60 min C/A Tribo Ratio** | 3.8 | 2.9 | 2.1 |

Toners 3 and 4 of the present disclosure have comparable charging results to control Toners 1. In fact, Toner 3 showed higher charge under both high temperature/high humidity conditions as well as under low temperature/low humidity conditions as compared to comparative Toner 1. Further, both Toners 3 and 4 of the present disclosure exhibit improved RH sensitivity over comparative Toners 1 as can be seen by the lower C/A tribo ratio for the inventive toners.

## Claims

1. A toner comprising:
at least one amorphous polyester;
at least one crystalline polyester; and
at least one ester wax;
wherein the at least one amorphous polyester and the at least one ester wax have a difference in solubility parameter of from about 0.1 to about 1.7.

2. The toner of claim 1, wherein the at least one amorphous polyester and the at least one ester wax have a difference in solubility parameter of from about 0.5 to about 1.4.

3. The toner of claim 1, wherein the ester wax is selected from the group consisting of monoester wax, diester wax, triester wax, and higher ester waxes, wherein high ester waxes comprise acid and alcohol components having six or more carbons, carnauba wax, rice bran wax, candelilla wax, sumac wax, jojoba oil, beeswax, montan wax, glyceride monostearate, glyceride distearate, pentaerythritol tetrabehenate; diethyleneglycol monostearate, dipropyleneglycol distearate, diglyceryl distearate, triglyceryl tetrastearate; sorbitan monostearate, cholesteryl stearate, and acid modified polyethylene wax, or
wherein the ester wax is behenyl behenate of the formula CH₃(CH₂)₂₀CO₂-(CH₂)₂₁CH₃, or wherein the ester wax is present in an amount of from about 1% to about 15% by weight of the toner.

4. The toner of claim 1, wherein the at least one amorphous polyester comprises a polyester selected from the group consisting of poly(propoxylated bisphenol A co-fumarate), poly(ethoxylated bisphenol A co-fumarate), poly(butyloxylated bisphenol A co-fumarate), poly(co-propoxylated bisphenol A co-ethoxylated bisphenol A co-fumarate), poly(1,2-propylene fumarate), poly(propoxylated bisphenol A co-maleate), poly(ethoxylated bisphenol A co-maleate), poly(butyloxylated bisphenol A co-maleate), poly(co-propoxylated bisphenol A co-ethoxylated bisphenol A co-maleate), poly(1,2-propylene maleate), poly(propoxylated bisphenol A co-itaconate), poly(ethoxylated bisphenol A co-itaconate), poly(butyloxylated bisphenol A co-itaconate), poly(co-propoxylated bisphenol A co-ethoxylated bisphenol A co-itaconate), poly(1,2-propylene itaconate); and
wherein the at least one crystalline polyester comprises a polyester selected from the group consisting of poly(ethylene-adipate), poly(propylene-adipate), poly(butylene-adipate), poly(pentylene-adipate), poly(hexylene-adipate), poly(octylene-adipate), poly(nonylene-adipate), poly(decylene-adipate), poly(undecylene-adipate), poly(dodecylene-adipate), poly(ethylene-succinate), poly(propylene-succinate), poly(butylene-succinate), poly(pentylene-succinate), poly(hexylene-succinate), poly(octylene-succinate), poly(nonylene-succinate), poly(decylene-succinate), poly(undecylene-succinate), poly(dodecylene-succinate), poly(ethylene-sebacate), poly(propylene-sebacate), poly(butylene-sebacate), poly(pentylene-sebacate), poly(hexylene-sebacate), poly(octylene-sebacate), poly(nonylene-sebacate), poly(decylene-sebacate), poly(undecylene-sebacate), poly(dodecylene-sebacate), poly(ethylene-dodecanedioate), poly(propylene-dodecanedioate), poly(butylene-dodecanedioate), poly(pentylene-dodecanedioate), poly(hexylene-dodecanedioate), poly(octylene-dodecanedioate), poly(nonylene-dodecanedioate), poly(decylene-dodecanedioate), poly(undecylene-dodecanedioate), poly(dodecylene-dodecanedioate), poly(ethylene-fumarate), poly(propylene-fumarate), poly(butylene-fumarate), poly(pentylene-fumarate), poly(hexylene-fumarate), poly(octylene-fumarate), poly(nonylene-fumarate), poly(decylene-fumarate), copolymers such as copoly(ethylene-fumarate)-copoly(ethylene-dodecandioate) and the like, alkali copoly(5-sulfoisophthaloyl)-copoly(ethylene-adipate), alkali copoly(5-sulfoisophthaloyl)-copoly(propylene-adipate), alkali copoly(5-sulfoisophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipate), alkali copoly(5-sulfo-isophthaloyl)-copoly(octylene-adipate), alkali copoly(5-sulfo-isophthaloyl)-copoly(ethylene-adipate), alkali copoly(5-sulfo-isophthaloyl)-copoly (propylene-adipate), alkali copoly(5-sulfo-isophthaloyl)-copoly(butylene-adipate), alkali copoly(5-sulfoisophthaloyl)-copoly(pentylene-adipate), alkali copoly(5-sulfo-isophthaloyl)-copoly(hexylene-adipate), alkali copoly(5-sulfo-isophthaloyl)-copoly(octylene-adipate), alkali copoly(5-sulfoisophthaloyl)-copoly(ethylene-succinate), alkali copoly(5-sulfoisophthaloyl)-copoly(propylene-succinate), alkali copoly(5 -sulfoisophthaloyl)-copoly(butylenes-succinate), alkali copoly(5 -sulfoisophthaloyl)-copoly(pentylene-succinate), alkali copoly(5-sulfoisophthaloyl)-copoly(hexylene-succinate), alkali copoly(5 -sulfoisophthaloyl)-copoly(octylene-succinate), alkali copoly(5 -sulfo-isophthaloyl)-copoly(ethylene-sebacate), alkali copoly(5-sulfo-isophthaloyl)-copoly(propylene-sebacate), alkali copoly(5-sulfo-isophthaloyl)-copoly(butylene-sebacate), alkali copoly(5-sulfo-isophthaloyl)-copoly(pentylene-sebacate), alkali copoly(5-sulfo-isophthaloyl)-copoly(hexylene-sebacate), alkali copoly(5-sulfo-isophthaloyl)-copoly(octylene-sebacate), alkali copoly(5-sulfo-isophthaloyl)-copoly(ethylene-adipate), alkali copoly(5-sulfo-isophthaloyl)-copoly(propylene-adipate), alkali copoly(5-sulfo-isophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipate); and
wherein the alkali comprises a metal selected from the group consisting of sodium, lithium, and potassium.

5. The toner of claim 1, wherein the at least one amorphous polyester comprises a poly(propoxylated bisphenol A co-fumurate) resin of the formula wherein m is from about 5 to about 1000; and
wherein the at least one crystalline resin is of the formula wherein b is from about 5 to about 200 and d is from about 5 to about 2000.

6. The toner of claim 1, wherein the amorphous polyester resin is present in an amount of from about 50 % to about 85 % by weight based upon the total weight of the toner, or
wherein the crystalline polyester resin is present in an amount of from about 5% to about 35% by weight based upon the total weight of the toner.

7. The toner of claim 1, comprising toner particles having a core with a shell thereover, or wherein the toner is an emulsion aggregation toner.

8. A process comprising:
contacting at least one amorphous polyester with at least one crystalline polyester and at least one ester wax in an emulsion comprising at least one surfactant, wherein the amorphous polyester and the at least one ester wax have a difference in solubility parameter of from about 0.1 to about 1.7, and an optional colorant;
aggregating the small particles to form a plurality of core particles;
contacting the core particles with an additional quantity of at least one amorphous polyester, at least one crystalline polyester, or a combination of at least one amorphous polyester and at least one crystalline polyester, to form a shell on the core particles;
coalescing the core-shell particles; and
optionally recovering the particles.

9. The process of claim 8, wherein the at least one amorphous polyester and the at least one ester wax have a difference in solubility parameter of from about 0.5 to about 1.4.

10. The process of claim 8, wherein the ester wax is selected from the group consisting of monoester wax, diester wax, triester wax, and higher ester waxes comprising acid and alcohol components wherein higher ester wax means having six or more carbons, carnauba wax, rice bran wax, candelilla wax, sumac wax, jojoba oil; beeswax; montan wax, glyceride monostearate, glyceride distearate, pentaerythritol tetrabehenate; diethyleneglycol monostearate, dipropyleneglycol distearate, diglyceryl distearate, triglyceryl tetrastearate; sorbitan monostearate, cholesteryl stearate, and acid modified polyethylene wax, or
wherein the ester wax is behenyl behenate of the formula CH₃(CH₂)₂₀CO₂-(CH₂)₂₁CH₃.

11. The process of claim 8, wherein the ester wax is present in an amount of from about 1% to about 15% by weight of the toner.

12. The process of claim 8, wherein the at least one amorphous polyester comprises a polyester selected from the group consisting of poly(propoxylated bisphenol A co-fumarate), poly(ethoxylated bisphenol A co-fumarate), poly(butyloxylated bisphenol A co-fumarate), poly(co-propoxylated bisphenol A co-ethoxylated bisphenol A co-fumarate), poly(1,2-propylene fumarate), poly(propoxylated bisphenol A co-maleate), poly(ethoxylated bisphenol A co-maleate), poly(butyloxylated bisphenol A co-maleate), poly(co-propoxylated bisphenol A co-ethoxylated bisphenol A co-maleate), poly(1,2-propylene maleate), poly(propoxylated bisphenol A co-itaconate), poly(ethoxylated bisphenol A co-itaconate), poly(butyloxylated bisphenol A co-itaconate), poly(co-propoxylated bisphenol A co-ethoxylated bisphenol A co-itaconate), poly(1,2-propylene itaconate); and
wherein the at least one crystalline polyester comprises a polyester selected from the group consisting of poly(ethylene-adipate), poly(propylene-adipate), poly(butylene-adipate), poly(pentylene-adipate), poly(hexylene-adipate), poly(octylene-adipate), poly(nonylene-adipate), poly(decylene-adipate), poly(undecylene-adipate), poly(dodecylene-adipate), poly(ethylene-succinate), poly(propylene-succinate), poly(butylene-succinate), poly(pentylene-succinate), poly(hexylene-succinate), poly(octylene-succinate), poly(nonylene-succinate), poly(decylene-succinate), poly(undecylene-succinate), poly(dodecylene-succinate), poly(ethylene-sebacate), poly(propylene-sebacate), poly(butylene-sebacate), poly(pentylene-sebacate), poly(hexylene-sebacate), poly(octylene-sebacate), poly(nonylene-sebacate), poly(decylene-sebacate), poly(undecylene-sebacate), poly(dodecylene-sebacate), poly(ethylene-dodecanedioate), poly(propylene-dodecanedioate), poly(butylene-dodecanedioate), poly(pentylene-dodecanedioate), poly(hexylene-dodecanedioate), poly(octylene-dodecanedioate), poly(nonylene-dodecanedioate), poly(decylene-dodecanedioate), poly(undecylene-dodecanedioate), poly(dodecylene-dodecanedioate), poly(ethylene-fumarate), poly(propylene-fumarate), poly(butylene-fumarate), poly(pentylene-fumarate), poly(hexylene-fumarate), poly(octylene-fumarate), poly(nonylene-fumarate), poly(decylene-fumarate), copolymers such as copoly(ethylene-fumarate)-copoly(ethylene-dodecanedioate) and the like, alkali copoly(5-sulfoisophthaloyl)-copoly(ethylene-adipate), alkali copoly(5-sulfoisophthaloyl)-copoly(propylene-adipate), alkali copoly(5 -sulfoisophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipate), alkali copoly(5-sulfo-isophthaloyl)-copoly(octylene-adipate), alkali copoly(5-sulfo-isophthaloyl)-copoly(ethylene-adipate), alkali copoly(5-sulfo-isophthaloyl)-copoly (propylene-adipate), alkali copoly(5-sulfo-isophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipate), alkali copoly(5-sulfo-isophthaloyl)-copoly(octylene-adipate), alkali copoly(5-sulfoisophthaloyl)-copoly(ethylene-succinate), alkali copoly(5-sulfoisophthaloyl)-copoly(propylene-succinate), alkali copoly(5-sulfoisophthaloyl)-copoly(butylenes-succinate), alkali copoly(5-sulfoisophthaloyl)-copoly(pentylene-succinate), alkali copoly(5-sulfoisophthaloyl)-copoly(hexylene-succinate), alkali copoly(5-sulfoisophthaloyl)-copoly(octylene-succinate), alkali copoly(5-sulfo-isophthaloyl)-copoly(ethylene-sebacate), alkali copoly(5-sulfo-isophthaloyl)-copoly(propylene-sebacate), alkali copoly(5-sulfo-isophthaloyl)-copoly(butylene-sebacate), alkali copoly(5-sulfo-isophthaloyl)-copoly(pentylene-sebacate), alkali copoly(5-sulfo-isophthaloyl)-copoly(hexylene-sebacate), alkali copoly(5-sulfo-isophthaloyl)-copoly(octylene-sebacate), alkali copoly(5-sulfo-isophthaloyl)-copoly(ethylene-adipate), alkali copoly(5-sulfo-isophthaloyl)-copoly(propylene-adipate), alkali copoly(5-sulfo-isophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipate); and
wherein the alkali comprises a metal selected from the group consisting of sodium, lithium, and potassium.

13. The process of claim 8, wherein the at least one amorphous polyester comprises a poly(propoxylated bisphenol A co-fumurate) resin of the formula wherein m is from about 5 to about 1000; and
wherein the at least one crystalline resin is of the formula wherein b is from about 5 to about 200 and d is from about 5 to about 2000.

14. The process of claim 8, wherein the amorphous polyester resin is present in an amount of from about 50 % to about 85 % by weight based upon the total weight of the toner.

15. The process of claim 8, wherein the crystalline polyester resin is present in an amount of from about 5% to about 35% by weight based upon the total weight of the toner.
